

United States Patent  
Boland et al.

[15] 3,668,302  
[45] June 6, 1972

[54] FLAME RETARDANT TEXTILE  
COVERED WIRE

[72] Inventors: Daniel Edmund Boland, Buffalo, N.Y.;  
Leonard S. Dewees, Baltimore, Md.;  
LeRoy M. Towsley, Berkeley Heights, N.J.

[73] Assignee: Western Electric Company, Incorporated,  
New York, N.Y.

[22] Filed: July 25, 1968

[21] Appl. No.: 747,757

[52] U.S. Cl. .... 174/121 A, 106/15 FP, 106/177,  
106/187, 106/196, 117/136, 117/232, 252/8.1

[51] Int. Cl. .... H01b 7/00, C09d 5/18

[58] Field of Search .... 106/187, 177, 196, 15 FP,  
117/136, 73, 78, 128.4, 232; 252/8.1; 174/121, 121  
FP

|           |         |                    |           |
|-----------|---------|--------------------|-----------|
| 1,981,132 | 11/1934 | Walsh et al. ....  | 106/177   |
| 2,126,850 | 8/1938  | Whitehead. ....    | 106/177   |
| 2,178,365 | 10/1939 | Brobst. ....       | 106/177   |
| 2,574,515 | 11/1951 | Walter et al. .... | 106/177 X |
| 2,618,568 | 11/1952 | Meyer et al. ....  | 106/177   |
| 2,675,327 | 4/1954  | Gearhart. ....     | 106/176   |
| 3,412,052 | 11/1968 | Taylor et al. .... | 106/15 X  |
| 3,515,565 | 6/1970  | Wood et al. ....   | 106/177   |

Primary Examiner—Lorenzo B. Hayes

Attorney—H. J. Winegar, R. P. Miller and A. J. Nugent

[56] References Cited

UNITED STATES PATENTS

1,936,985 11/1933 Lommel et al. .... 106/177 UX

[57] ABSTRACT

A textile served wire coated with a flame retardant lacquer comprised essentially of a mixture, by weight, of 100 parts cellulose acetate base, 35 parts tricresyl phosphate plasticizer, 42.5 parts tris (2, 3 - dibromopropyl) phosphate flame retardant, and 128.5 parts acetone solvent.

4 Claims, 1 Drawing Figure



PATENTED JUN 6 1972

3,668,302



INVENTORS  
Daniel E. Boland  
Leonard S. Dewees  
LeRoy M. Towsley

*Sommer & Weber*

ATTORNEYS

## FLAME RETARDANT TEXTILE COVERED WIRE

## BACKGROUND OF THE INVENTION

## 1. Field of the Invention

This invention relates to improvements in flame retardant compositions, and more particularly, to a new and improved flame retardant lacquer for coating textile covered wire, and to new and improved textile covered wire having its covering coated with such flame retardant lacquer.

In the production of textile served wire, which is particularly adapted for use in the so-called U-type distributing frames employed in telephone exchanges, it is common practice to extrude a flexible polyvinyl chloride insulating layer over the conductor wire. Where feasible, this insulating layer incorporates a suitable flame retardant plasticizer. This operation is followed by wrapping of the cotton textile serving over the insulation, whereupon the served wire is passed through an impregnating chamber wherein a substantially transparent lacquer coating is applied under pressure to prevent unraveling or fraying of the serving, while permitting visibility of the underlying serving for identification purposes, the thickness of the coating being controlled by passage of the wire out of the chamber through a rubber die having a central aperture of a predetermined size. The emerging coated wire is continuously wound and air dried on a series of capstans prior to being reeled.

## 2. Description of the Prior Art

A typical prior art lacquer formulation employed in the above process is as follows:

| Ingredients         | Parts by Weight |
|---------------------|-----------------|
| Cellulose Acetate   | 100             |
| Tricresyl Phosphate | 20              |
| Triphenyl Phosphate | 35              |
| Dimethyl Phthalate  | 30              |
| Dibutyl Phthalate   | 8.75            |
| Acetone             | 148 (approx.)   |

While this lacquer possesses the physical characteristics necessary for use in the wire coating process and is effective in serving the desired purposes of visibility of the serving and of preventing unraveling and fraying of such serving, it nevertheless is not sufficiently flame retardant. This is true particularly because of the presence of the phthalate plasticizers, which are flammable and tend to negate the flame retardant characteristics of the phosphate plasticizers.

## SUMMARY OF THE INVENTION

Accordingly, it is a primary object of the present invention to provide a new and improved flame retardant lacquer which is just as feasible for use in the aforesaid wire coating process and just as effective in permitting visibility of the serving and in preventing unraveling and fraying of such serving, as the aforesaid lacquer. To this end, the present lacquer is comprised essentially of a mixture of a base, a plasticizer, a flame retardant and a solvent present in the following proportions by weight: 100 parts of derivative of cellulose (preferably cellulose acetate) as the base, between about 25 and 35 parts of derivative or cresylic acid and phosphorous oxychloride (preferably 35 parts tricresyl phosphate) as the plasticizer, between about 40 and 45 parts of a brominated monomeric triaryl phosphate (preferably 42.5 parts of tris (2,3-dibromopropyl) phosphate as the flame retardant, and between about 120 and 150 parts of dimethyl ketone, ethyl methyl ketone, ethanol or methanol (preferably 128.5 parts of dimethyl ketone; i.e., acetone) as the solvent.

Another primary object is to provide a new and improved textile covered wire having its covering coated with the aforesaid flame retardant lacquer.

Additional objects and advantages of the invention will become apparent upon consideration of the following detailed description and accompanying drawing, wherein:

## BRIEF DESCRIPTION OF THE DRAWING

The single FIGURE is an enlarged side elevational view of a textile served wire coated with the inventive flame retardant lacquer and constitutes a preferred embodiment of the invention.

## DETAILED DESCRIPTION OF THE PREFERRED EMBODIMENT

10 Referring to the drawing, the textile served wire is generally indicated at 10, and includes a central conductor 12 surrounded by an insulating layer 14 preferably formed of fire retardant plasticized polyvinyl chloride, a preferably cotton and color coded textile serving 16 wrapped around insulating layer 14 which in turn is impregnated with and surrounded by the inventive flame retardant lacquer coating 18. The coating is substantially transparent for visibility of the underlying serving.

20 Wire 10 is particularly adapted for use in the so-called U-type distributing frames in telephone exchanges, and for this purpose its various elements have the following typical physical characteristics. Conductor 12 is made of 22AWG gauge copper wire, insulating layer 14 has an average wall thickness of 8 mils, serving 16 is made of 20/1 cotton yarn, and the weight of lacquer coating 18 ranges between about 60 and 80 milligrams per foot of wire, with the preferred weight being about 70 milligrams.

25 In producing wire 10, insulating layer 14 is extruded over conductor 12 and serving 16 is wrapped around layer 14, such serving preferably being provided with a differently colored tracer thread (not shown) for identification purposes. The textile served wire is then unreeled and passed through an impregnating chamber (not shown) into which the lacquer is injected under pressure to form coating 18, the thickness and weight of which is controlled by passage of the coated wire out through a rubber sizing die (not shown) of the desired diameter. As the coated wire leaves the chamber it is wound continuously over a series of moving capstans (not shown) to air dry lacquer coating 18 and is rereeled.

30 In order to successfully process wire 10, it is imperative that lacquer coating 18 have the following physical properties. First, it must be sufficiently lubricious to permit smooth passage through the sizing die. Secondly, it must be sufficiently fast drying to permit winding on the capstans and reels without adhesion of the wire coating thereto or to itself. Third, it must have sufficient film flexibility to prevent the lacquer from cracking on the wire, particularly when wound on the reels.

35 45 50 While the prior art coating referred to above does possess these physical characteristics, it is not sufficiently flame retardant. Accordingly, the principal problem to overcome was to eliminate the flammable phthalate plasticizers in order to obtain the desired flame retardance, while still maintaining the other physical characteristics necessary for successful coating of the wire. After extensive experimentation, which also involved replacement of the fire retardant phenyl phosphate fire retardant plasticizer with more tricresyl phosphate because of its greater lubricity, the following formulation was developed as a preferred embodiment of the invention.

## EXAMPLE

| Ingredients                       | Parts by Weight |
|-----------------------------------|-----------------|
| Cellulose Acetate                 | 100             |
| Tricresyl Phosphate               | 35              |
| Tris(2,3-Dibromopropyl) Phosphate | 42.5            |
| Dimethyl Ketone (Acetone)         | 128.5           |

70 Comparative flame retardance tests were made between wires which had the physical characteristics described above for wire 10, and were otherwise identical, except for the lacquer coating. In one test, wire 10, with the inventive

lacquer coating of the example, was placed on several shelves on a small distributing frame and a 4-inch diameter dish of alcohol was placed below a shelf and ignited. The wire withstood 12 minutes exposure to the alcohol flames with only slight burning and was self-extinguished immediately after the alcohol was consumed. In contrast, wire having the aforesaid prior art lacquer coating ignited after about 1 minute in the alcohol and the fire slowly spread both horizontally and vertically.

In another test using the distributing frame mentioned above and wire 10 with lacquer 18, the horizontal side of the frame was ignited and produced a strong fire extending over several shelves. Wire 10 burned only in the flames in the region of the terminals and the fire did not propagate along the wire. In a similar test using wire with the prior art lacquer, the flames from the terminals spread along the wire and enlarged the fire.

Accordingly, it is evident that wire coated with the inventive lacquer exhibits greatly improved flame retardance over that coated with the prior art lacquer. At the same time, the inventive lacquer coating 18 also possesses the physical characteristics of lubricity, fast drying and film flexibility necessary for efficient and effective processing of the wire during and after coating, drying and rereeling. The coated wire 10 also has been found to possess better handling characteristics than the same wire coated with the prior art lacquer, the improvement being attributed to a smoother outer surface.

Although the formulation of the example represents a preferred embodiment of the inventive lacquer, this formulation can be varied within certain limits and still produce an acceptable flame retardant lacquer coating. For example, while cellulose acetate is preferred because of its electrical insulating properties, other suitable derivatives of cellulose such as cellulose formate among the esters and ethyl cellulose among the ethers, may be used as the base.

The preferred derivative of cresylic acid and phosphorous oxychloride for use as the plasticizer is tricresyl phosphate, because it not only provides the needed die lubrication and film flexibility but also contributes to flame retardance. However, the amount of this ingredient may vary between about 25 and 35 parts per 100 parts of base.

As for the flame retardant, a partially brominated monomeric triallyl phosphate is usable, but the fully brominated phosphate of the example is preferred because of its greater flame retardance. This ingredient also functions as a secondary plasticizer and may vary in amount between about 40 and 45 parts per 100 parts of base.

While the quantity of solvent may range between about 120 and 150 parts per 100 parts of base, and other solvents such as

ethyl methyl ketone, ethanol or methanol may be substituted, dimethyl ketone (i.e.; acetone) is preferred because it is the most volatile for minimizing drying time and least toxic for minimizing exposure of personnel to toxic fumes.

Within the aforesaid ranges, the percentage of each ingredient is critical from the standpoint of both proper operation of the coating process and obtaining the maximum practical flame retardance. If too much flame retardant is used; i.e., more than about 45 percent of the base, the formulation will cause adhesion to the capstans and will not run. If the plasticizer exceeds about 35 percent of the base, it will contribute to the adhesion problems. Should the ratio of the flame retardant to the plasticizer exceed about 9/5 (45/25), film flexibility is adversely affected, while a ratio below about 8/7 (40/35) undesirably reduces flame retardance. This critical property is also adversely affected if the ratio of the combined percentage of the flame retardant and plasticizer to the base falls below about 0.65/1 (65/100). Likewise, the ratio of the total of the other ingredients to the solvent should not exceed about 3/2 (180/120) nor should it be less than about 1.1/1 (165/150), in order to control the viscosity for obtaining a proper amount of lacquer coating on the wire, the optimum amount being obtained with the preferred ratio of the example; i.e. about 1.48/1 (177.5/128.5).

While the inventive lacquer described herein is especially suitable for coating the textile covered wire referred to herein, it also may be used to coat other objects or may be formed into filaments, ribbons, sheets, or other convenient forms by any suitable method known in the art.

What is claimed is:

1. A textile covered wire having its covering coated with a substantially transparent flame retardant lacquer consisting essentially of a dried mixture of a base, a plasticizer, a flame retardant and a solvent present prior to drying in the following proportions by weight: 100 parts of a derivative of cellulose as the base, between about 25 and 35 parts of tricresyl phosphate as the plasticizer, between about 40 and 45 parts of tris(2,3-dibromopropyl phosphate as the flame retardant, and between about 120 and 150 parts of dimethyl ketone, ethyl methyl ketone, ethanol or methanol as the solvent.
2. The wire of claim 1 wherein said base is cellulose acetate.
3. The wire of claim 2 wherein said solvent is dimethyl ketone.
4. The wire of claim 3 wherein said base, plasticizer, flame retardant and solvent are present prior to drying in the following proportions: 100 parts cellulose acetate, 35 parts tricresyl phosphate, 42.5 parts tris (2, 3 - dibromopropyl) phosphate, and 128.5 parts dimethyl ketone.

\* \* \* \* \*

# UNITED STATES PATENT OFFICE CERTIFICATE OF CORRECTION

Patent No. 3,668,302 Dated June 6, 1972

Inventor(s) Daniel E. Boland-Leonard S. DeWees-Leroy M. Towsley

It is certified that error appears in the above-identified patent and that said Letters Patent are hereby corrected as shown below:

[Redacted]

In the specification, Column 4, line 35, Claim 1 insert following the word "cellulose", --selected from the group consisting of cellulose esters and cellulose ethers--.

Signed and sealed this 14th day of January 1975.

(SEAL)  
Attest:

McCOY M. GIBSON JR.  
Attesting Officer

C. MARSHALL DANN  
Commissioner of Patents

[Redacted]